

[54] CERAMIC-METAL SYSTEMS BY INFILTRATION

[75] Inventors: George E. Gazza, Sudbury, Mass.; Michael W. Lindley, Holton Heath, England

[73] Assignees: The United States of America as represented by the Secretary of the Army, Washington, D.C.; by said Gazza; The Secretary of State for Defence Ministry of Defence, London, England; by said Lindley

[22] Filed: Nov. 9, 1972

[21] Appl. No.: 305,038

[52] U.S. Cl. .... 29/123 B, 29/182.1, 117/22, 117/54, 117/61, 117/131, 117/135.1, 117/160, 117/169 AR, 264/60

[51] Int. Cl. .... C03c 17/00, C04b 41/00

[58] Field of Search .... 117/22, 54, 61, 98, 119, 117/121, 123 B, 160, 169 A, 169 R, 135.1, 131; 29/182.1; 75/202; 51/309; 264/60

[56] References Cited

UNITED STATES PATENTS

1,913,373 6/1933 Golyer ..... 75/202 X

|           |        |                     |            |
|-----------|--------|---------------------|------------|
| 2,581,252 | 1/1952 | Goetzel et al. .... | 29/182.1 X |
| 2,581,253 | 1/1952 | Ellis et al. ....   | 29/182.1 X |
| 2,612,443 | 9/1952 | Goetzel et al. .... | 29/182.1 X |
| 2,672,426 | 3/1954 | Grubel et al. ....  | 117/121    |
| 3,457,051 | 7/1969 | Bergna. ....        | 75/202 X   |
| 3,718,441 | 2/1973 | Landingham. ....    | 29/182.1 X |
| 3,725,015 | 4/1973 | Weaver. ....        | 75/202 X   |

Primary Examiner—William D. Martin

Assistant Examiner—Shrive P. Beck

Attorney, Agent, or Firm—Robert P. Gibson

[57]

ABSTRACT

This invention covers ceramic-metal compositions fabricated by infiltrating a porous ceramic compact with a molten metal impregnant. A cold pressed compact of silicon boride, aluminum boride, boron, and (aluminum boride-boron) were each positioned between powdered aluminum in a vacuum furnace which enabled the molten aluminum to infiltrate into the porous ceramic by capillary action. In addition, a porous ceramic compact of aluminum boride was similarly infiltrated with silicon.

6 Claims, 2 Drawing Figures



Al B<sub>12</sub>—Al (500X)

PATENTED FEB 4 1975

3,864,154



Al B<sub>12</sub> — Al (500X)

FIG. 1



Al B<sub>12</sub> — Si (500X)

FIG. 2

**CERAMIC-METAL SYSTEMS BY INFILTRATION**

The invention described herein may be manufactured, used, and licensed by or for the Government for governmental purposes without the payment us use of any royalty thereon.

**BACKGROUND OF THE INVENTION**

This invention relates to the production of ceramic-metal materials, and more particularly to production by the infiltration of a porous cold pressed ceramic compact with a molten metal.

**SUMMARY OF THE INVENTION**

It is an object of the present invention to provide and disclose the fabrication of ceramic-metal materials comprising the filtration of a molten metal into a porous ceramic compact.

It is a further object of the invention to provide and disclose a ceramic-metal material comprising a uniform dispersion of the metal in the ceramic.

It is a further object of the invention to provide and disclose a ceramic-metal material having each component in a continuous phase.

It is a further object of the present invention to provide and disclose a ceramic-metal material exhibiting ductility.

It is a further object of the present invention to provide and disclose a ceramic-metal material which is generally hard and non-ductile.

Other objects and a fuller understanding of the invention may be ascertained from the following description and claims taken in conjunction with the accompanying drawings in which:

**BRIEF DESCRIPTION OF THE DRAWING**

FIG. 1 is a photomicrograph of a cross-sectional area microstructure of an  $\text{AlB}_{12}$ -Al infiltrated compact.

FIG. 2 is a photomicrograph of a cross-sectional area microstructure of an  $\text{AlB}_{12}$ -Si infiltrated compact.

**DESCRIPTION OF THE PREFERRED EMBODIMENTS**

Other objects and a fuller understanding of the invention may be ascertained from the following description and claims.

In an illustrative example, a cold pressed compact of  $\text{AlB}_{12}$  powder (minus 325 mesh), 1 inch in diameter and 0.3 inch thick, which was formed by applying 17,000 psi pressure to the powder in a cold pressing die, was utilized. A graphite crucible having an I.D. of 1 1/2 inch was lined with 0.005 inch thick grafoil sheet. Six grams of aluminum powder were placed at the bottom of the crucible and lightly tamped. The cold pressed  $\text{AlB}_{12}$  compact was placed on the aluminum powder. Six additional grams of aluminum powder were positioned on top of the  $\text{AlB}_{12}$  powder compact and a grafoil lid was placed over the top of the crucible. The crucible, loaded with  $\text{AlB}_{12}$  compact "sandwiched" between the aluminum powder, was placed in a vacuum furnace. The furnace was evacuated to approximately  $10^{-5}$  torr and the crucible was heated to 500°C and held at this temperature 1 1/2 hours to permit outgassing. The temperature was subsequently raised to 1,100°C and maintained for a period of 3 hours. At

this temperature, the molten aluminum easily penetrated into the porous  $\text{AlB}_{12}$  compact.

The process was repeated utilizing silicon in lieu of the aluminum. The procedure was identical with the exception that the outgassing temperature was 750°C for a period of 1 1/2 hours and the infiltration temperature was 1,500°C for a period of 2 hours.

In addition to the above ceramic-metal materials,  $\text{SiB}_6$ -Al; B-Al;  $\text{B}_4\text{C}$ -Al/Si; and  $\text{AlB}_{12}$ -B-Al materials have been prepared utilizing the above conditions. The last material consisted of a ceramic skeleton comprised of 60% by weight  $\text{AlB}_{12}$  and 40% by weight boron, impregnated with aluminum metal. For  $\text{B}_4\text{C}$ -Al/Si, silicon was added to the aluminum and this combination was impregnated into  $\text{B}_4\text{C}$ , the silicon acting as a wetting agent.

TABLE

| 20 | SYSTEM (g/cc)           | DENSITY<br>RUPTURE | MOD. OF<br>MOD. | ELASTIC            |
|----|-------------------------|--------------------|-----------------|--------------------|
|    | B-Al                    | 2.32               | 17,500 psi      | $16.7 \times 10^6$ |
|    | $\text{AlB}_{12}$ -Al   | 2.59               | 47,900 psi      | $32.3 \times 10^6$ |
|    | $\text{AlB}_{12}$ -B-Al | 2.47               | 30,000 psi      | $19.5 \times 10^6$ |

Densities of the ceramic-metal compositions were within the range of about 2.3 to about 2.7 g/cc. Possible uses of the ceramic-metal material include ceramic armor, ceramic composite bearings and wear-resistant specialized materials.

Although we have described our invention with a certain degree of particularity, it is understood that the present disclosure has been made by way of example and that numerous modifications may be resorted to in the ways of components and reaction conditions, etc. without departing from the spirit and scope of the invention.

Having described our invention, we claim:

1. A ceramic-metal composition consisting of a metal impregnated into a porous ceramic compact by infiltration, selected from the group consisting of:

| 45 | CERAMIC              | METAL IMPREGNANT |
|----|----------------------|------------------|
| a) | $\text{SiB}_6$ -     | Al               |
| b) | $\text{AlB}_{12}$ -  | Al               |
| c) | $\text{AlB}_{12}$ -  | Si               |
| d) | B -                  | Al               |
| e) | $\text{AlB}_{12}$ -B | - Al             |

2. A material in accordance with claim 1 wherein the ceramic-metal material is  $\text{SiB}_6$ -Al.

3. A material in accordance with claim 1 wherein the ceramic-metal material is  $\text{AlB}_{12}$ -Si.

4. A material in accordance with claim 1 wherein the ceramic-metal material is B-Al.

5. A material in accordance with claim 1 wherein the ceramic-metal material is  $\text{AlB}_{12}$ -B-Al.

6. A ceramic-metal composition in accordance with claim 1 wherein the ceramic-metal composition is  $\text{AlB}_{12}$ -Al.

\* \* \* \* \*